

Nov. 9, 1948.

A. J. MORWAY ET AL

2,453,153

LUBRICATING GREASE

Filed Dec. 6, 1947



John C. Zimmer  
Arnold J. Morway Inventors

By J. L. Small Attorney

## UNITED STATES PATENT OFFICE

2,453,153

## LUBRICATING GREASE

Arnold J. Morway, Clark Township, Union County, and John C. Zimmer, Union, N. J., assignors to Standard Oil Development Company, a corporation of Delaware

Application December 6, 1947, Serial No. 790,219

14 Claims. (Cl. 252—29)

1

This invention relates to lubricants, and in particular to highly viscous lubricating compositions, specifically lubricating greases, having definite yield values.

The accompanying drawing represents a graphical comparison of the relation of viscosity with temperature of two compositions having the same consistency (penetration) at 77° F., one composition, indicated at A, prepared according to the present invention and the other composition, indicated at B, being a prior art composition consisting essentially of a sodium soap and mineral oil. The comparative uniformity of composition A over a wide temperature range is readily apparent.

In the past, lubricating greases, solid and semi-solid, have usually been prepared by employing various metal soaps as thickeners, incorporating them in mineral oils either as pseudo solutions or as fine dispersions. These grease compositions have in general shown a thinning out or liquefaction or marked tendency toward liquefaction upon heating. At high temperatures, such compositions have shown the effect of the swelling of the soap in the oil, causing considerable thickening with unpredictable viscosity changes, varying with different soaps, until the melting point of the soap was reached, at which point the lubricant approached the viscosity of the oil constituent.

In prior art grease compositions, where soap was used as the thickener, apparent viscosity was usually found to be dependent upon the viscosity of the mineral oil and consistency was dependent upon the amount and type of soap. It was generally found, moreover, that the viscosity of the grease decreased with increasing shear rates and at high rates of shear the viscosity approached that of the mineral oil base, even at moderate temperatures, and more so at higher temperatures. It has heretofore been difficult or impossible to make a single grease composition which would be suitable for use over a relatively wide temperature range because of the unpredictable viscosity behavior. This problem has been an active one but until the present invention, no satisfactory solution appears to have been proposed. In grease compositions of the present invention, unique and desirable viscosity characteristics are obtained.

For many years, certain carbon blacks have been incorporated in mineral oils and other viscous oily materials for various purposes. It has been recognized that for most purposes the most desirable carbon blacks are those which impart

2

an intense black hue with a minimum thickening effect. Printing inks, which are essentially oily suspensions of carbon black demand a very intense color, as do other analogous compositions. In the present invention, acetylene black, which has a dull greyish appearance and therefore, undesirable for the above uses, has been found to have unexpected and pronounced thickening properties in refined mineral lubricating oils and to be particularly suitable for the preparation of lubricating grease compositions having excellent temperature-consistency properties.

In the preparation of lubricating grease or grease-like compositions with acetylene black, from 3 to 20% by weight of the black may be employed. Particularly desirable greases are prepared by incorporating 5 to 18% by weight of the acetylene black in mineral oils of the lubricating oil range. The amounts of acetylene black required to prepare grease compositions of a given body and consistency are much smaller than the amounts necessary with other types of carbon black. For example, a grease containing only 11% acetylene black in mineral oil has the same consistency, i. e. resistance to penetration, as a grease composition prepared with 18% of ordinary channel black in the same oil. In addition, the other required properties of the grease are superior, in the case of that prepared from acetylene black. In these lubricating grease compositions, the mineral oil constituent may be derived from a paraffin, naphthene or mixed base crude and may have a viscosity ranging from that of a light mineral oil of about 50 Saybolt Universal seconds at 100° F. to that of a heavy cylinder oil of viscosity of about 1000 Saybolt Universal seconds at 210° F.

In preparing the lubricating grease or grease-like compositions containing acetylene black and mineral oils, acetylene black has an additional practical advantage. It is only necessary to mix the acetylene black into the oil by ordinary stirring means. The compositions thus prepared from acetylene black and mineral oil have a smooth viscous consistency and a relatively uniform distribution of the black throughout the oil. In order to prepare lubricating compositions from other carbon blacks, such as channel black, a high degree of mechanical working of the black in the oil is necessary, as for example, passage of the mixture through a paint mill. Furthermore, with the compositions prepared from these blacks, it is almost or quite impossible to obtain as uniform distribution of the black in the oil as in the case of acetylene black.

Acetylene black is also found to be an advantageous constituent of lubricating compositions on account of the relative ease of removal of the grease composition from hands and clothing. In contrast to the channel blacks, for example, which have intense color and are very difficult to remove from skin and clothing, the acetylene black has an important and practical advantage.

*Example 1*

In the preparation of a lubricating composition containing 12% by weight of acetylene black and 88% of a naphthene base lubricating oil having a viscosity of 70 Saybolt Universal seconds at 210° F. a small portion of the oil was initially added to a typical grease kettle equipped with side-scraping paddles and the acetylene black was added. The speed of the paddles was controlled so as to obviate loss of the added carbon. The balance of the oil was added in small portions to the mass undergoing agitation and was worked gradually into the mixture to prevent lumping of the black. The composition thus prepared had a smooth paste consistency and a firm grease-like appearance, an A. S. T. M. penetration (worked) at 77° F. of 300, and under the conditions of test for the A. S. T. M. dropping point did not show a melting point.

For purposes of comparison a sodium soap grease was prepared having the same consistency as the above grease at 77° F. This composition was prepared from the following ingredients:

|                                                                                  | Percent |
|----------------------------------------------------------------------------------|---------|
| Rapeseed oil                                                                     | 22      |
| Flake caustic soda                                                               | 4.75    |
| Sodium petroleum sulfonates                                                      | 0.5     |
| Mineral lubricating oil (Coastal oil of 55 Saybolt seconds viscosity at 210° F.) | 71.75   |
| Phenyl alpha naphthylamine                                                       | 1       |

To prepare this grease, the rapeseed oil, sodium sulfonates and one-third of the mineral oil were placed in a grease kettle and heated to 150° F. The caustic soda was then thoroughly stirred in as a 30% aqueous solution and the mixture was heated to 225° F. until substantially all the water had been removed. The balance of the mineral oil was added and the temperature raised to 500° F. after which the source of heat was removed and the grease was allowed to cool to 275° F. while being paddle stirred. The phenyl alpha naphthylamine was then added and the grease was worked and cooled until its temperature was lowered to 200° F. where it was then filtered and packaged. This grease had an A. S. T. M. penetration of 300 and an A. S. T. M. dropping point of 440° F.

As suggested above, in the drawing the two compositions mentioned above are compared graphically as to the variation of their apparent viscosities with temperature at constant rate of shear; graph A relating to the acetylene black composition of Example 1 and graph B relating to the sodium soap composition described above. In this graphical analysis, presented on a semi-logarithmic scale, apparent viscosity in poises is plotted against temperature. Apparent viscosity was measured by means of a pressure viscosimeter.

Inspection of the graphs shows that over the temperature range of 150° F. to 340° F. the apparent viscosity of the grease composition of the present invention is relatively uniform, varying from 15 to 10 poises, whereas over the same tem-

perature range, the apparent viscosity of the sodium soap grease varies from 38 to a low point of about 8 poises and then increases to a high of about 80 poises.

The abrupt fluctuations occurring in the soap thickened lubricant are considered to be caused by solvation and swelling of the soap in oil with rising temperature resulting in a change in grease structure which in turn causes a sudden increase in apparent viscosity. In the composition of the present invention, no apparent changes occur in the grease structure with increasing temperature. Thus, the composition of the present invention is a smooth uniform product with good lubricating properties. Changes in grease structure from a smooth consistency to a fibrous ropey material such as occur with typical soap thickened greases result in lubrication failures and this is undesirable.

*Example 2*

Another composition was prepared generally similar to that of Example 1. In this case, 11% by weight of acetylene black was thoroughly mixed in 89% of a naphthene base lubricating oil having a viscosity of 70 Saybolt Universal seconds at 210° F. The composition thus prepared had an A. S. T. M. penetration (worked) at 77° F. of 286 and under the conditions for the A. S. T. M. dropping point did not show a melting point.

*Example 3*

18% of a commonly available channel black was dispersed in the same naphthene base lubricating oil as used in Example 2. In dispersing this material to obtain maximum body, it was necessary to employ a paint mill, the mixture being passed several times through the mill. The composition had an A. S. T. M. penetration (worked) at 77° F. of 292 and there was no apparent melting point.

To compare the oxidation stability of compositions thickened respectively with channel black and with acetylene black, prepared as described in Examples 2 and 3, portions of each were subjected to the standard Norma-Hoffmann Bomb Oxidation Test. In this test, the composition is subjected to oxygen under pressure of 110 lbs. per sq. inch at 210° F. and the time required for a five pound drop in oxygen pressure is noted. The following results were obtained:

|    |                                    |
|----|------------------------------------|
| 50 | No. hours to give 5# pressure drop |
|    | Coastal mineral lubricating oil    |
|    | Same oil plus 11% acetylene black  |
|    | Same oil plus 18% channel black    |

55 Compositions of superior lubricating characteristics are prepared by the incorporation in the acetylene black thickened grease of a thickening agent in an amount between 0.1% and 2% by weight. Suitable thickening agents are polyisobutylene, rubber, or other such linear hydrocarbon polymers. Instead of linear hydrocarbon type polymeric material, an ester polymer, such as a methacrylate polymer or a dilinoleate of a polyhydric alcohol, particularly of a glycol, may be employed. The use of polybutene in combination with a methacrylic acid ester polymer is particularly advantageous. These thickening agents are usually incorporated in the grease by adding an oil solution of the thickening agents to the grease and thoroughly mixing. Rubber latex or swollen gum rubber, with or without a stabilizer or oxidation inhibitor or an oil solution of natural or synthetic rubber may also be employed in the composition. The polymers present in these compositions have little effect in

60 65 70 75

general on the consistency but impart adhesive-ness and stringiness to lubricants particularly de-sirable for lubricants employed in connection with reciprocating or other such mechanisms which involve shock effects in their cycle of operation. These polymeric materials also aid in preventing leakage and spattering of the lubri-cant from shock systems.

It has also been found that lubricants highly advantageous for high temperature and high pressure lubrication purposes may be prepared by compounding mineral oils, acetylene black and extreme pressure additives of either the oil-soluble or oil-insoluble type. Thus, when 5% to 15% by weight of acetylene black is blended with a mineral oil to give a grease-like structure, 0.5% to 10% of any of the oil-insoluble, high temper-ature, extreme pressure additives such as phosphorus sesquisulphide, powdered lead, free sul-fur, zinc oxide, titanium oxide and graphite may be incorporated in the mass to prepare highly desirable extreme pressure lubricants. As an illustration in this connection the following ex-ample is presented. Rubber or other polymeric thickeners may be added, as suggested above.

*Example 4*

8 parts by weight of acetylene black was mixed into 92 parts by weight of a steam refined cylin-der oil of Mid-continent origin of 180 Saybolt Universal seconds viscosity at 210° F. (lubricant A). The acetylene carbon black was dispersed in the mineral oil by simple mixing in a grease kettle to prepare a smooth, semi-fluid mass. To this mixture was added 2.0% of a solution con-taining 6% of high molecular weight (m. w. 60,000 to 100,000) polyisobutylene in mineral oil, and 0.5% finely powdered phosphorus sesquisulfide ( $P_4S_3$ ) and thoroughly mixed again in the grease kettle. The resultant product (lubricant B) was a semi-fluid, stringy, cohesive and adhesive product. This product had a small but definite yield value and under low shearing stresses was fluid, but upon removal of the stress the product reset to a nonfluid mass. Under the conditions of the Almen test, the following data were obtained:

| Lubricant | Almen Test<br>Gradual Loading<br>(pounds carried) | Pin Condition                 | Shock Loading<br>Weight Applied<br>at one time<br>(pounds carried) | Pin Condition                             |
|-----------|---------------------------------------------------|-------------------------------|--------------------------------------------------------------------|-------------------------------------------|
| A.....    | 4,000                                             | Sheared.....                  | 2,000                                                              | .....                                     |
| B.....    | 15,000                                            | Excellent (like<br>original). | 15,000                                                             | Sheared.<br>Excellent (like<br>original). |

Of the oil-soluble extreme pressure additives lead oleate and lead naphthenate are the most commonly employed, and usually in amounts be-tween 5% and 20% by weight. In order to im-part a relatively high load-carrying ability, such other extreme pressure agents as the sulfurized, chlorinated or sulfo-chlorinated mineral oil, chlo-rine-containing sulfides, polysulfides, xanthates, mercaptans, sulfurized or sulfo-chlorinated fatty oil, esters, olefins, diolefins, chlorinated waxes or chlorinated aromatic hydrocarbons, and amines, may be blended in the mineral oil-carbon black composition.

In these compositions the extreme pressure ad-ditives are mixed directly with the acetylene black and mineral oil. In the case of mineral oils thick-ened with soaps, on the other hand, preliminary treatment of the chemically active compounds employed as the extreme pressure additive is gen-erally necessary to reduce chemical reaction be-tween the additive and the soap constituent.

Thus, the extreme pressure additives, such as free sulfur, phosphorus sesquisulfide and molyb-denum sulfide are effective in smaller concentra-tions in compositions prepared mainly from min-eral oils and acetylene black than in compositions prepared mainly from mineral oils and soaps.

As additional examples of the invention, the following may be cited:

*Example 5*

16 parts by weight of acetylene black were mixed with 84 parts of a high quality paraffin base lubricating oil having a viscosity of about 80 S. S. U. at 210° F., and a viscosity index of 103. 15 The resulting grease was of excellent texture, stable against oil separation and of firm solid consistency.

*Example 6*

20 For a comparison between acetylene black and ordinary channel black, 16 parts by weight of channel black were mixed with 84 parts of a high quality light colored low pour naphthenic base oil having a viscosity of about 70 S. S. U. at 25 210° F. and a viscosity index of 39. The result-ing grease was of fair texture, and of soft con-sistency, showing a marked tendency to oil separa-tion after about 10 days storage.

*Example 7*

30 For a general comparison between graphite and acetylene black, 16 parts by weight of graphite were added to 84 parts by weight of a lubricat-ing oil identical with that of Example 6. A sus-pension was produced by mixing but the graph-ite rapidly settled out of the oil, leaving the up-35 per three-fourths of the volume as a substan-tially clear liquid oil and the bottom one-fourth a thick precipitate of graphite within a few min-utes. The composition had no grease-like struc-ture or texture, although the freshly mixed com-position was quite thick.

*Example 8*

To determine the utility of acetylene black as

55 a thickener in oils of other than mineral base origin, 16 parts by weight of acetylene black were added to 84 parts of castor oil and thoroughly mixed. The resulting composition was a soft but smooth and uniform grease of good appearance and good physical stability. No noticeable oil separation occurred after standing for 30 days. The grease was considerably softer in consist-60 ency, however, than that of Example 5 which contained the same amount of acetylene black.

*Example 9*

8 parts by weight of acetylene black were mixed with 92 parts of a very light lubricating oil, used 70 widely also as a transformer oil. The oil was a highly refined low pour oil having a viscosity at 100° F. of only 57 S. S. U. and a viscosity of about 35 S. S. U. at 210° F. It had a viscosity index of 65 64. The resulting grease composition was of excellent solid body and consistency and showed 75 no tendency to oil separation.

*Example 10*

8 parts by weight of acetylene black were mixed into 92 parts of the same high quality light colored mineral base lubricating oil as used in Examples 6 and 7 (70 S. S. U. viscosity at 210° F.). The resulting grease was of good consistency, fairly soft but of excellent texture, and showed a very slight tendency to oil separation after 10 days storage.

*Example 11*

5 parts by weight of acetylene black were mixed with 95 parts of the same light transformer type oil as described in connection with Example 9 above (57 S. S. U. viscosity at 100° F. and 35 S. S. U. at 210° F.). The resulting grease was quite soft but of definite grease-like structure and of good texture. Some oil separation was noted after 10 days storage.

*Example 12*

5 parts by weight of acetylene black were mixed with 95 parts of a light lubricating oil identical with that used in Examples 6, 7 and 10 (70 S. S. U. viscosity at 210° F.). The resulting composition had a definite grease-like structure but was very soft, being of semi-solid consistency. It showed little tendency, however, to oil separation after 10 days storage.

*Example 13*

3 parts by weight of acetylene black were mixed with 97 parts of the same lubricating oil as described above in connection with Examples 6, 7, 10 and 12, above (70 S. S. U. at 210° F.). The resulting composition was a very thin lubricant, quite liquid at ordinary room temperatures, but having a uniform texture and grease-like appearance. There was no apparent tendency for the oil to separate from the acetylene black or for the acetylene black to precipitate, even though the composition was quite liquid. In this respect the contrast with the graphite thickened composition of Example 7, and even with the channel black composition of Example 6 which showed a notable oil separation was marked.

From the foregoing examples it appears to be clear that acetylene black may be used as the bodying or grease-like structure forming agent in various mineral oils over a wide range of concentrations. The oils also may vary widely in viscosity. For greases of definitely solid consistencies about 5% by weight appears to be the minimum requirement for acetylene black, based on the total composition. The maximum has not been exactly determined but it would appear that not more than 20% acetylene black by weight, based on the total composition, would ordinarily be used in greases. The oil, which is preferably mineral base oil but may also be vegetable or other oil of comparable viscosity and viscosity index, or mixtures thereof, with mineral oil, should have a viscosity of at least about 50 S. S. U. at 100° F., or about 35 S. S. U. at 210° F., and may go as high as 1000 S. S. U. at 210° F. if desired. In any case, where a true grease or grease-like composition is desired, the quantity of acetylene black should be adjusted, taking into consideration the viscosity and viscosity index of the oil, to provide sufficient thickening that a definite structure or body is produced in the composition.

Such additives as the metal sulfonates, metal phenates, and the metallic derivatives of phenol sulfides or of organo-thiophosphate or the reaction products of phosphorus sulfides with metal

sulfonates, metal phenates, metal phenol sulfides and the like, may also be employed. Also, such addition agents as elementary sulfur, the phosphorus sulfides, the mercaptans, the mercaptides, sulfides, disulfides, xanthates, carbamates, polysulfides, xanthate polysulfides, their metal derivatives, etc. may be employed in minor proportions. These various addition agents may be employed with corrosion inhibitors such as amine condensation products, amines, alkanol amines, ammonium bases or onium compound or metal soaps. Oxidation inhibitors such as phenyl alpha naphthylamine and di-tert.-butyl-p-cresol may also be used.

15 This application is a continuation-in-part of application Serial No. 729,922, which was filed February 21, 1947, and which in turn was a continuation-in-part of applications Serial Nos. 570,780, 570,782 (forfeited) and 570,783 (now abandoned) filed December 30, 1944.

20 What is claimed is:

1. A semi-solid to solid lubricating grease comprising lubricating oil with 5 to 20% by weight, based upon the finished composition, of acetylene 25 black incorporated therein, the quantity of acetylene black being sufficient to impart a grease-like consistency and body to said oil.

2. A semi-solid to solid lubricant according to 30 claim 1 in which the acetylene black is present from about 9% to about 18% by weight of the lubricating oil.

3. A semi-solid to solid lubricating grease composition comprising a mineral base oil having a viscosity from about 50 Saybolt Universal seconds 35 at 100° F. to about 1000 Saybolt Universal seconds at 210° F. and from about 5% to about 20% by weight, based on the total composition, of acetylene black, the quantity of said acetylene black being sufficient to impart a grease-like 40 consistency and body to said oil.

4. A semi-solid to solid lubricant according to 45 claim 3 in which the acetylene black is present from about 9% to about 18% by weight of the mineral oil.

5. A lubricating composition comprising a mineral lubricating oil compounded with 5 to 20% acetylene black to form a grease-like substantially solid structure in which also a linear, high molecular weight, substantially oil soluble 50 polymer is added in an amount between 0.1 and 2% by weight of the mineral oil.

6. An improved lubricating composition according to claim 5 in which the linear, high molecular weight, substantially oil-soluble polymer 55 is polybutene.

7. An improved lubricating composition according to claim 5 in which the linear, high molecular weight, oil-soluble polymer is a polymerized ester.

8. A non-melting adhesive lubricating grease comprising 5 to 20% of acetylene black and 2% of a 6% solution of a linear, high molecular weight, oil-soluble polymer compounded with mineral oil of a viscosity between 50 S. S. U. at 60 100° F. and 1000 S. S. U. at 210° F.

9. A non-melting adhesive lubricating grease according to claim 8 in which the linear, high molecular weight, substantially oil-soluble polymer is polybutene.

10. A non-melting adhesive lubricating grease according to claim 8 in which the linear, high molecular weight, substantially oil soluble polymer is a methacrylate polymer.

11. A lubricating composition consisting essen-

tially of 11% acetylene black dispersed in naphthenic lubricating oil of 70 Saybolt Universal seconds at 210° F. and 0.1 to 2% of polybutene.

12. A high temperature extreme pressure semi-solid to solid lubricating quasi composition consisting essentially of lubricating oil thickened to a grease-like consistency and body with 5 to 15% by weight, based on the total composition, of acetylene carbon black, said grease also containing about 0.5 to 10% by weight of an oil insoluble phosphorus sulfide finely dispersed therein as a high temperature extreme pressure agent.

13. Composition as in claim 12 wherein said phosphorus sulfide is phosphorus sesquisulfide.

14. Composition as in claim 12 to which is added a small amount of a tacky relatively inert organic polymer as a stringiness agent.

ARNOLD J. MORWAY.  
JOHN C. ZIMMER.

## REFERENCES CITED

The following references are of record in the file of this patent:

## UNITED STATES PATENTS

| Number    | Name    | Date          |
|-----------|---------|---------------|
| 1,880,987 | Silhavy | Oct. 4, 1932  |
| 2,349,058 | Swenson | May 16, 1944  |
| 2,356,365 | Wright  | Aug. 22, 1944 |

## OTHER REFERENCES

Uses and Applications of Chemicals and Related Materials, 1939, page 148, Thomas C. Gregory, Reinhold Pub. Corp., New York, N. Y. (Copy in Division 64.)

Canadian Chem. & Met., vol. 17, May 1933, Article entitled, "Acetylene Carbon Black" by Charles Kaufmann, pages 93 to 95.

Petroleum Refiner, March 1944, Article entitled, "Carbon Black" by J. F. Gallie, page 106.